

## UNITED STATES PATENT OFFICE

2,603,423

METHOD FOR THE REMOVAL OF SULFUR  
FROM SPONGE IRONRussell C. Buehl, Edgewood, Pa., assignor to the  
United States of America as represented by the  
Secretary of the InteriorNo Drawing. Application January 6, 1947,  
Serial No. 720,326

5 Claims. (Cl. 241—14)

(Granted under the act of March 3, 1883, as  
amended April 30, 1928; 370 O. G. 757)

1

The invention described herein may be manufactured and used by or for the Government of the United States for governmental purposes without the payment to me of any royalty thereon in accordance with the provisions of the act of April 30, 1928 (Ch. 460, 45 Stat. L. 467).

This invention relates to the removal of sulfur from metals reduced from their ores at temperatures sufficiently low so that melting does not occur and, in particular, to the removal of sulfur from sponge iron.

In order to produce certain grades of steel, especially tool steels, it is necessary to use iron having a very low sulfur content, generally less than 0.06 percent sulfur by weight. Sponge iron has been found to be a desirable melting stock for the production of steels, especially tool steels in electric arc furnaces, but its sulfur content is often undesirably high for this application. Sponge iron can be produced economically and the sulfur content can be controlled by the use of lime, limestone, or dolomite as described in U. S. Patent 2,380,406 and in the co-pending application of Buehl et al. Serial No. 778,452, filed October 7, 1947, now United States Patent No. 2,495,225. However, these sulfur control agents increase the cost of production of the material and do not always yield sponge iron with as low a sulfur content as is desired. The process herein described may be employed to advantage to further lower the sulfur content of sponge iron made with the use of sulfur control agents.

Accordingly, it is an object of this invention to provide an easy and economical method for the removal of sulfur from sponge iron. It is another object of the invention to provide a good cheap melting stock of low sulfur iron for the production of tool steels and other special alloys. Other objects and advantages will be obvious or will appear hereinafter.

These objects and advantages are accomplished in accordance with this invention by abrading the surface of sulfur bearing sponge iron and separating therefrom the fines thereby broken from said surface, whereby a low sulfur bearing sponge iron product is produced.

The method accordingly comprises a means of removing sulfur from sponge iron or other metals reduced from their ores at temperatures below the melting point of the constituents.

In operation, a sulfur bearing sponge iron product is subjected to suitable abrading treatment such as selective grinding, roll crushing, tumbling, and the like. By this action the brittle

surface layer is broken off as powdered fines without appreciably decreasing the size of the malleable sponge iron particles. Grinding equipment that involves the impact of the iron particles at high velocities has been found to accomplish the abrading in a satisfactory manner and is presently preferred. Thereafter, the fines or the broken surface particles, are separated from the sponge iron particles by suitable particle classifying means such as sieving, magnetic separation, sink and float separation, air classification, and the like. The more massive particles so obtained are found to have a considerably lower sulfur content than the initial sponge iron product.

15 The following examples show how the invention may be carried out, but it is not limited thereto. Percentages are by weight unless specified to the contrary.

20

## Example I

A sample of sponge iron containing 0.061 percent sulfur was mechanically sieved to remove the minus 200 mesh particles. This sieving lowered the sulfur content of the sponge iron to 0.051 percent with a loss of only 1.9 percent of the iron content of the sample.

## Example II

30 A sponge iron containing 0.061 sulfur was ball milled for 10 minutes then sieved. The removal of the minus 325 mesh particles lowered the sulfur content of the sponge iron to 0.053 percent with a loss of 3.1 percent of the iron; and the 35 removal of the minus 200 mesh particles lowered the sulfur content of the sponge iron to 0.045 percent with a loss of 8.2 percent of the iron.

## Example III

40 A sample of magnetically concentrated sponge iron containing 0.148 percent sulfur was passed through roll crushers which flattened the particles somewhat without much grinding action. The roll crushed product was reseparated on a 45 magnetic separator. This lowered the sulfur content to 0.075 percent.

As shown in the foregoing description and examples, the sulfur content of sponge iron can easily and economically be decreased by abrading the surface of the sponge iron product and removing the fines which have been broken from the surface.

50 While the invention has been particularly described employing specific abrading means, it is 55 not limited thereto.

While the invention has been particularly described employing specific separating or classifying means, it is not limited thereto.

Since many apparently widely differing embodiments of the invention will occur to one skilled in the art, the invention is not limited to the specific details illustrated and described, and various changes may be made therein without departing from the spirit and scope thereof.

What is claimed is:

1. The method of producing low sulfur content sponge iron which comprises treating the iron ore at a temperature below the melting point of the constituents of said ore in the presence of a solid carbonaceous material as the reducing agent and a desulfurizing agent selected from the group consisting of dolomite, lime and limestone to produce sponge iron particles having a closely adhering, brittle surface coating of high sulfur content basic slag, then abrading the surface of the so produced sponge iron particles to remove the brittle surface layer, and then separating from the abraded sponge iron particles the fines of high sulfur content slag which have been broken from the surface of said particles.

2. The method of claim 1 wherein the abrading is accomplished by ball mill grinding.

3. The method of claim 1 wherein the abrading is accomplished by high velocity impact grinding.

4. The method of claim 1 wherein the abrading is accomplished by roll crushing.

5. The method of claim 1 wherein the abrading is accomplished by ball mill grinding and the separating is accomplished by sieving to remove the fines.

RUSSELL C. BUEHL.

#### REFERENCES CITED

10. The following references are of record in the file of this patent:

#### UNITED STATES PATENTS

| Number       | Name             | Date          |
|--------------|------------------|---------------|
| 15 957,157   | Goltra           | May 3, 1910   |
| 1,822,647    | Dubbert          | Sept. 8, 1931 |
| 2,232,696    | Earle            | Feb. 25, 1941 |
| 2,240,718    | Schiffman et al. | May 6, 1941   |
| 2,264,204    | Heckett          | Nov. 25, 1941 |
| 20 2,287,663 | Brassert         | June 23, 1942 |
| 2,352,712    | Heckett          | July 4, 1944  |
| 2,380,406    | Buehl            | July 31, 1945 |
| 2,381,022    | Wulff            | Aug. 7, 1945  |
| 2,462,900    | Riott            | Mar. 1, 1949  |

#### 25 FOREIGN PATENTS

| Number  | Country       | Date         |
|---------|---------------|--------------|
| 466,048 | Great Britain | May 21, 1937 |